

## UNITED STATES PATENT OFFICE

2,109,271

## VITREOUS ENAMELED PRODUCTS

Daniel E. Krause, Columbus, Ohio, assignor, by  
mesne assignments, to Monsanto Chemical  
Company, a corporation of Delaware

No Drawing. Application October 5, 1936,  
Serial No. 104,063

10 Claims. (Cl. 91—73)

This invention relates to a vitreous enameled product. It furthermore relates to an improved ferrous base alloy suitable for use in the manufacture of vitreous enameled products.

5 One object of the present invention is the provision of an enameled product having increased strength at elevated temperatures. Another object is the provision of an enameled product providing increased resistance to chipping of the 10 enamel layer. A further object is the provision of an enameled sheet having increased resistance to deflection and warpage both at enameling temperatures and at ordinary temperatures. Still another object of this invention is the provision 15 of an improved ferrous base alloy suitable for use in the manufacture of vitreous enameled objects. Other objects and advantages of my invention will become apparent from the following description and claims.

20 In the art of enameling sheet iron and sheet steel the various ground and cover coats are fired in continuous or box type furnaces at temperatures ranging from a minimum of about 1400° F. to a maximum of about 1650° F. The base 25 metal is therefore heated to these temperatures at which its strength is comparatively low. Small articles either drawn or stamped from sheet may through their design promote sufficient rigidity to withstand deformation, but massive articles such as panelings, refrigerator linings and shells, table tops, stove parts and other related articles do not offer sufficient rigidity 30 through design and therefore introduce difficult problems for the enameler in seeking to avoid warpage and sagging. Many of the larger enameled articles also act as load bearing members in the assembled product. For that reason they demand increased strength at normal temperatures.

40 The ferrous materials now employed for vitreous enameling comprise the commercial pure iron, known as enameling iron, and the various grades of enameling and ordinary steel. Their composition limits are about as follows:

| Constituent     | Enameling iron | Enameling steel | Ordinary steel |
|-----------------|----------------|-----------------|----------------|
|                 | Percent        | Percent         | Percent        |
| 50 Carbon.....  | 0.01-0.035     | 0.035-0.15      | 0.15-0.25      |
| Silicon.....    | 0.01-0.07      | 0.01-0.10       | 0.01-0.10      |
| Manganese.....  | 0.02-0.06      | 0.25-0.50       | 0.35-0.55      |
| Sulphur.....    | 0.01-0.05      | 0.02-0.05       | 0.02-0.05      |
| Phosphorus..... | 0.004-0.01     | 0.005-0.05      | 0.02-0.05      |

55 Enameling iron may at times contain as much

as 0.10 to 0.3% manganese to eliminate susceptibility to red-shortness and to lower production costs.

It is general knowledge that enameling iron affords fewer defects and rejections on enameling principally because of its lower carbon content. Its lower strength on the other hand makes it more apt to warp and sag unless supported well during enameling. In contrast, the enameling steels are stronger at room temperatures, 10 though not materially stronger at the enameling temperatures, and are more prone to contain defects in the enameled surface. Moreover, the steels pass through an eutectoid transformation which marks the beginning of the change from 15 alpha to gamma iron. This transformation, the  $A_1$  arrest, or the lower critical, occurs in the usual commercial steels at close to 1340° F. The conversion of alpha to gamma iron involving large volume changes is completed at the upper critical or the  $A_3$  arrest temperature. Commercial 20 enameling iron, due to its relative freedom from carbon has no  $A_1$  arrest. It changes to gamma iron at what is virtually the  $A_3$  arrest for pure iron. This is at 1670° F., a temperature above 25 that normally used in enameling; hence the gamma transformation may not occur on firing enameling iron.

The  $A_3$  arrest for enameling steels varies from 1670° F. for those of low carbon to 1340° F. for 30 those of eutectoid steel compositions. It is evident from this and from the fact that the conversion begins at above 1340° F. that part or all of the alpha iron will be transformed to gamma iron on heating and that this gamma iron must 35 revert to alpha iron on cooling from enameling temperatures. A marked contraction in volume occurs during the transformation on heating; an equally marked expansion occurs during the transformation on cooling with the result that 40 in vitreous enameling of steels no adequate provision for supporting the articles against the above mentioned volume changes can be provided for and the finished articles are subjected to considerable distortion and warpage. 45

While the resistance to sagging of enameling iron has improved through the development of enamels of lower maturing temperatures, an improvement in the resistance of enameling steels to the warpage and distortion arising from contraction and expansion during phase changes 50 cannot be accomplished as readily by the same procedure.

I have now found that the resistance to warpage and distortion is greatly improved by alloy- 55

ing the enameling sheet with phosphorus. Furthermore, I have found that the strength of enameling sheet at high temperatures is improved by phosphorus; and therefore its resistance to sagging is improved. I have also discovered that phosphorus does not enhance such common defects encountered in enameling iron or steel as copper heading, blistering, reboiling and fish-scaling, nor does it affect the adherence or bonding qualities of enamels when its content is under 0.40%. I have also discovered that resistance to chipping of the enamel is also augmented through strengthening the base metal.

I have employed as much as 1% phosphorus in 15 enameling sheet with excellent results. As the adherence or bond of the enamel to the base metal was somewhat less at phosphorus contents above 0.40% I have preferred to use phosphorus contents ranging from 0.1% to 0.35% in 20 sheet requiring good enamel adherence. The enameling stock containing more than 0.4% phosphorus, because of its strength and stiffness, is better suited for flat panels and for ware requiring no severe deep drawing operations as 25 well as for ware in which the requirement for exceptionally good enamel adherence is unimportant.

The strengthening effect of phosphorus in steel at normal testing temperatures has been recognized for some time. Tensile properties of phosphorus bearing 22 gauge enameling iron and steel sheet as set forth in the accompanying table illustrate this point. The enameling iron contained 0.01 to 0.02% carbon, 0.05 to 0.06% manganese, 0.02 to 0.07% silicon, about 0.03% sulphur, and phosphorus as shown in the table. The enameling steel contained 0.12 to 0.13% carbon, 0.08 to 0.10% silicon, 0.5-0.6% manganese, and about 0.04% sulphur, with phosphorus as shown.

| Type of enameling sheet | Percent phosphorus | Tensile strength lbs./sq. in. | Yield strength lbs./sq. in. | Elongation in 2" percent |
|-------------------------|--------------------|-------------------------------|-----------------------------|--------------------------|
| 45 Iron                 | 0.008              | 42,000                        | 30,000                      | 32                       |
|                         | 0.10               | 49,500                        | 45,000                      | 30                       |
|                         | 0.20               | 57,000                        | 52,000                      | 28                       |
|                         | 0.30               | 64,000                        | 55,000                      | 28                       |
|                         | 0.49               | 71,500                        | 62,500                      | 22                       |
|                         | 0.75               | 81,500                        | 73,000                      | 17                       |
|                         | 1.07               | 91,000                        | 83,000                      | 14                       |
| 50 Steel                | 0.008              | 53,000                        | 42,000                      | 20                       |
|                         | 0.17               | 64,500                        | 40,500                      | 21                       |
|                         | 0.31               | 75,000                        | 49,000                      | 21                       |

The sheet was normalized before testing.

It is evident from the listed properties that 55 phosphorus from the standpoint of strength is as effective as carbon. In other respects it is more satisfactory than carbon. Carbon, for example, does not improve the strength at elevated temperatures to the same extent as phosphorus. It likewise reduces the  $A_3$  arrest temperature which causes more alpha iron to transform during firing. Carbon also increases the number of such defects as blistering, reboiling and copper heading in the 60 enameling surface.

65 Phosphorus, on the other hand, improves the high temperature tensile properties and raises the  $A_3$  arrest temperature of both enameling iron and steel. In the case of enameling steel 0.2 to 0.3% phosphorus so effectively reduces the amount of 70 alpha iron that is converted during firing of the enamel as to virtually eliminate the distortion and warpage which prevail as a result of this conversion when steel is enameled. Moreover, phosphorus does not intensify the occurrence of 75 common defects appearing in enameled ware. I

found it advantageous, therefore, to employ phosphorus wherever high strength and excellent enameling qualities in sheet are desired.

My invention, therefore, embraces an improved enameling iron and steel of superior strength at room and at elevated temperatures and of superior resistance to sagging, distortion and warping. In accomplishing these improvements I alloy from 0.10% to 1% phosphorus to the iron and steel. For ordinary purposes the quantity of 1 phosphorus is below 0.35% and above 0.10%. Where exceptional strength is required in enameled ware I may employ more than 0.35% phosphorus and in fact increase the phosphorus to a maximum of 1%.

The general accepted maximum percentage of phosphorus in vitreous enameling sheet is 0.04% yet most sheet-makers prefer to keep it under 0.02%. For large vitreous enameled parts where flatness of the finished part is of importance an extra low-metallloid, open hearth steel graded as special vitreous enameling sheet is being used. It retains its flatness under firing better than normal steel and it gives better enameling results. This sheet, which may be classified as enameling iron, has a total metallloid content including carbon, silicon, manganese, sulphur and phosphorus not in excess of 0.15% of which less than 0.01% is phosphorus.

The prior art teaches that phosphorus serves 30 no useful purpose in the manufacture of sheet other than to prevent sticking on rolling and argues that it must be kept to a minimum in enameling sheet.

Contrary to these teachings I found that phosphorus serves as an important element in enameling sheet by adding strength, thereby reducing sagging and warpage and improving the retention of flatness on firing, by providing a more suitable base metal for the more brilliant and 40 more permanent higher melting point enamels, and by increasing the temperature of the upper critical point. All these are accomplished without detriment to enameling qualities provided the phosphorus is below 0.40%. 45

In steel, phosphorus is particularly advantageous from another score since it raises the  $A_3$  arrest temperature to a point where the inversion of alpha to gamma iron becomes of little importance insofar as producing much distortion 50 and warpage in the enameled article. The  $A_3$  arrest temperature on heating a steel with 0.15-0.20% carbon and 0.03% phosphorus was 1540° F. This was raised to 1585° F. on increasing the phosphorus to 0.1%, to 1650° F. on increasing 55 the phosphorus to 0.2% and to 1700° F. on increasing the phosphorus to 0.29%. Thus the marked rise in temperature of the  $A_3$  arrest with an increase in phosphorus content is apparent.

This rise in the  $A_3$  arrest temperature resulting from the addition of phosphorus is also of marked importance in enameling irons containing manganese. Each 0.01% manganese reduces the  $A_3$  arrest temperature about 2.5° F. so that with 0.1 to 0.3% manganese in enameling iron 65 its  $A_3$  arrest temperature may be from 25° to 75° F. lower than it is for iron of low manganese content. The reduction is sufficient to bring the arrest temperature below the maximum enamel maturing temperature and hence sufficient to 70 promote the alpha-gamma transformation during the firing of refractory enamels. The  $A_3$  arrest temperatures for enameling iron containing 0.004%, 0.11%, and 0.20% phosphorus were 1670° F., 1780° F., and 1950° F., respectively. 75

In a previous application, Serial No. 81,338, filed May 22, 1936, I have shown the strengthening effect of phosphorus in iron and steel for service at elevated temperatures. In this respect it is superior to carbon. As a result of alloying phosphorus to enameling iron and steel I have found the increase in strength at elevated temperatures is reflected in greater resistance of sheet to sagging. This was demonstrated by 10 enameling 4" by 10" specimens of 22 gauge sheet which were coated with 9.8 to 11.8 grams of ground coat enamel and fired at 1580° F. for 4 minutes. They were supported on the ends leaving an unsupported span of 8½ inches in the center free to sag. The deflections after firing provided a measure of the resistance to sagging. In a series of enameling irons containing from 0.005% to 0.40% phosphorus these measured permanent deflections were as follows:

|    | Phosphorus content in per cent | Permanent deflection in inches |
|----|--------------------------------|--------------------------------|
| 25 | 0.005                          | 0.10                           |
|    | 0.11                           | 0.00                           |
|    | 0.21                           | 0.02                           |
| 20 | 0.40                           | +0.02 (arched upward)          |

The reduction in sagging as shown by these tests is due to the phosphorus content of the sheet and to the influence of phosphorus on high temperature strengths of sheet.

An enameling steel such as I prefer to use for the manufacture of enameled sheets may have the following composition, where enamel adherence is not of major importance:

|              | Percent              |
|--------------|----------------------|
| Phosphorus   | between 0.10 and 1.0 |
| Carbon       | do 0.01 and 0.25     |
| Silicon      | do 0.01 and 0.10     |
| 40 Manganese | do 0.02 and 0.55     |
| Sulphur      | do 0.01 and 0.05     |
| Iron         | Balance              |

Where enamel adherence is of importance I prefer to use between 0.10 and 0.40% of phosphorus in a steel which otherwise has an analysis as given above.

An enameling iron such as I prefer to use for the manufacture of enameled sheets may have the following composition where enamel adherence is not of major importance:

|            | Percent              |
|------------|----------------------|
| Phosphorus | between 0.10 and 1.0 |
| Carbon     | do 0.01 and 0.035    |
| 55 Silicon | do 0.01 and 0.07     |
| Manganese  | do 0.02 and 0.30     |
| Sulphur    | do 0.01 and 0.05     |
| Iron       | Balance              |

Where enamel adherence is of importance I prefer to use between 0.10 and 0.40% of phosphorus in an iron which otherwise has an analysis as given above.

Having now particularly described my invention and the manner in which it is to be carried out, I desire that it not be limited except as indicated by the prior art, or as particularly pointed out in the claims.

What I claim is:

1. A vitreous enameled article comprising a layer of vitreous enamel vitrified upon the surface of a steel sheet said steel containing from 0.1 to 1.0% of phosphorus, the balance being iron containing the usual impurities ordinarily occurring in enameling steel.

2. A vitreous enameled article comprising a layer of vitreous enamel vitrified upon the surface of a steel sheet, said steel containing 0.1% to 1.0% of phosphorus, 0.01 to 0.25% carbon, 0.01 to 0.10% silicon, 0.02 to 0.55% manganese, 0.01 to 0.05% sulphur, the remainder being substantially iron. 5

3. A vitreous enameled article comprising a layer of vitreous enamel vitrified upon the surface of an iron sheet, said iron sheet containing 10 from 0.1 to 1.0% of phosphorus, 0.01 to 0.035% carbon, 0.01 to 0.07% silicon, 0.02 to 0.30% manganese, 0.01 to 0.05% sulphur, the remainder being substantially iron.

4. A vitreous enameled article comprising a 15 layer of vitreous enamel vitrified upon the surface of a steel sheet, said steel containing from 0.1 to 0.35% phosphorus, 0.01 to 0.25% carbon, 0.01 to 0.10% silicon, 0.02 to 0.55% manganese, and 0.01 to 0.05% sulphur, the balance being sub- 20 stantially iron.

5. A vitreous enameled article comprising a layer of vitreous enamel vitrified upon the surface of an iron sheet, said iron containing from 0.1 to 0.35% phosphorus, 0.01 to 0.035% carbon, 25 0.01 to 0.07% silicon, 0.02 to 0.30% manganese, 0.01 to 0.05% sulphur, the remainder being substantially iron.

6. A vitreous enameled article comprising a coating of vitreous enamel, vitrified upon the 30 surface of a ferrous alloy sheet, said sheet containing from 0.1 to 1.0% phosphorus, 0.01% to 0.25% carbon, 0.01 to 0.10% silicon, 0.02% to 0.55% manganese and 0.01 to 0.05% sulfur alloyed therewith, the balance being substantially 35 iron.

7. A vitreous enameled article comprising a layer of vitreous enamel vitrified upon the surface of a steel sheet, said steel containing sufficient phosphorus alloyed therewith to raise the 40 upper critical temperature of said steel above the maturing temperature of said vitreous enamel.

8. A vitreous enameled article comprising a 45 layer of vitreous enamel vitrified upon the surface of an iron sheet, said iron containing between 0.01% and 0.25% carbon together with the usual alloying elements in iron sheets employed for enameled articles and containing, in addition, sufficient phosphorus alloyed with said iron to 50 raise the upper critical temperature of said iron to above the maturing temperature of said enamel.

9. A vitreous enameled article comprising a 55 layer of vitreous enamel vitrified upon the surface of a steel containing between 0.01% and 0.25% carbon together with the usual alloying elements and impurities in steel sheets employed for enameled steels, and containing, in addition, sufficient phosphorus alloyed therewith to raise 60 the upper critical temperature of said steel to above the maturing temperature of said enamel.

10. A vitreous enameled article possessing an extended plane surface comprising a layer of vitreous enamel vitrified upon the surface of a 65 ferrous alloy in sheet form containing from 0.01 to 0.25% carbon and containing in addition sufficient phosphorus alloyed therewith to retain said plane surface substantially without sagging or warping, at temperatures approximating the 70 maturing temperature of the said enamel.

DANIEL E. KRAUSE.